

A. F. SULZER,  
PHOTOGRAPHIC FILM,  
APPLICATION FILED FEB. 21, 1921.

1,432,368.

Patented Oct. 17, 1922.



WITNESS

*James K. Stewart.*

INVENTOR  
*Albert F. Sulzer,*  
BY *R. L. Stinchfield*

ATTORNEY

## UNITED STATES PATENT OFFICE.

ALBERT F. SULZER, OF ROCHESTER, NEW YORK, ASSIGNOR TO EASTMAN KODAK COMPANY, OF ROCHESTER, NEW YORK, A CORPORATION OF NEW YORK.

## PHOTOGRAPHIC FILM.

Application filed February 21, 1921. Serial No. 446,784.

To all whom it may concern:

Be it known that I, ALBERT F. SULZER, a citizen of the United States of America, residing at Rochester, in the county of Monroe and State of New York, have invented certain new and useful Improvements in Photographic Films, of which the following is a full, clear, and exact specification.

This invention relates to photographic film and to the base or support for such film. The principal object of this invention is to provide a film having the qualities desirable in commercial practice, which will likewise be so made that markings due to electrical discharges are prevented or very greatly minimized. Other objects will hereinafter appear.

In the handling of sensitive photographic film, particularly that of the usual kind which includes a nitrocellulose support or base, characteristic lines or patches sometimes appear on development, due to electrical discharges, which occur when the film is manipulated. While the defect may crop out during manufacture, it is particularly troublesome in the motion picture field, especially when making negative film strips. It is customarily referred to as "static" and will be so designated hereinafter.

While several changes in motion picture cameras have been suggested for preventing static, it is highly desirable to prevent the trouble by a proper constitution of the film, so that the latter may be employed in any commercial apparatus without the necessity of special precautions.

I have discovered that film having strong anti-static properties may be prepared by adding certain substances to the nitrocellulose film base or support, and then coating the rear face of it with a suitable anti-static layer. Thus I may coat film of the kind indicated in the co-pending applications of Paul C. Seel, Serial Nos. 434,353 and 434,354, both filed Dec. 31, 1920, on the rear face or surface opposite the sensitive photographic coating with an anti-static insoluble backing. This backing may, for example, be of cellulose acetate, or cellulose ether, or various mixtures of these substances with each other or with cellulose nitrate, as indicated in U. S. Patent No. 1,232,702, Lovejoy, July 10, 1917, and the applications of Albert F. Sulzer, Serial

Nos. 446,782 and 446,783 both filed Feb. 55 21, 1921.

In the accompanying drawing the figure is a sectional view on an exaggerated scale of a film embodying my invention.

The support 1 carries the sensitive layer 60 2 on one face and the insoluble anti-static backing 3 on the other.

A photographic film comprising a photographically sensitive layer and a nitrocellulose support containing hygroscopic metallic salts, together with water and certain co-operating agents is a very useful product, and static is prevented with great effectiveness. But when the hygroscopic substances and the water are present in the 70 higher amounts in their range of proportions, there may be a tendency in certain warm and damp climates for the water to appear on the rear face of the film and affect the sensitive emulsion with which it contacts when the film is coiled up. By coating the rear face of the film with an anti-static insoluble backing, I not only provide the film with a double insurance against static, but at the same time remove any risk 80 of this injurious sweating. There is also a stronger tendency for the water to remain sealed in the film base in dry climates.

By way of illustration, the nitrocellulose base may be manufactured from a dope 85 comprising 100 parts of nitrocellulose, 250 parts of acetone, 250 parts of methyl alcohol, 40 parts of fusel oil, 10 parts of camphor, 1 part of sodium hypophosphite, 5 parts of glycerin and 5 parts of water. 90 Equivalents may be substituted and the proportions widely varied, as indicated in the applications of Paul C. Seel hereinabove referred to.

Upon this hygroscopic anti-static film 95 base there is coated the usual gelatino-silver haloid sensitive emulsion. On the face opposite the emulsion there is deposited a cellulosic anti-static layer or coating which may, for instance, be cellulose acetate of 100 the kind which is soluble in acetone. It is very thin. The coating may be made from a weak solution of the acetate in a mixture of acetone and ethyl alcohol, the latter being sufficiently diluted, so that the composition is clear and the cellulose acetate not precipitated.

The coating may likewise be of cellulose

ether, in which case I prefer a dilute composition of the type indicated in the Sulzer applications hereinabove mentioned. For instance, I may use a composition comprising 5 90 parts of ethyl cellulose, 600 parts of ethyl alcohol, 900 parts of chloroform and 3000 parts of acetone. Of course, equivalent coatings disclosed in the Lovejoy patent and in the Sulzer applications may be 10 substituted. All such coatings are substantially non-sweating,—that is, their outer surfaces remain satisfactorily free from moisture even in a hot and humid atmosphere.

15 Having thus described my invention, what I claim as new and desire to secure by Letters Patent is:

1. A photographic film comprising a sensitive coating and an anti-static hygroscopic 20 nitrocellulose support therefor, the face of said support opposite said sensitive coating being provided with a non-sweating insoluble anti-static coating.

2. A photographic film comprising a sensitive coating and an anti-static nitrocellulose support therefor, which contains a hygroscopic substance and water, the base of said support opposite said sensitive coating being provided with a non-sweating anti-static coating. 25 30

3. A photographic film comprising a sensitive coating and an anti-static hygroscopic nitrocellulose support therefor, the face of said support opposite said sensitive coating being provided with a cellulosic anti-static 35 non-sweating coating.

4. A photographic film comprising a sensitive coating and an anti-static nitrocellulose support therefor, which contains an inert hygroscopic metallic salt, glycerin and 40 water, the face opposite said sensitive coating being provided with a coating of cellulose acetate.

Signed at Rochester, New York, this 15th day of February, 1921.

ALBERT F. SULZER.